

1

3,788,957

## ELECTRODEPOSITION OF CHROMIUM

Ian Robert Arthur Christie, Twickenham, and John Joseph Bernard Ward, Welling, England, assignors to International Lead Zinc Research Organization, Inc., New York, N.Y.

No Drawing. Filed Oct. 2, 1972, Ser. No. 293,860  
Claims priority, application Great Britain, Sept. 30, 1971,  
45,669/71

Int. Cl. C23b 5/06, 5/46

U.S. Cl. 204—51

13 Claims

### ABSTRACT OF THE DISCLOSURE

An improved method and an improved electrolyte solution for providing a chromium coating on a metal substrate. The metal coatings are provided by electrodepositions from solutions comprising water, dimethylformamide, trivalent chromium ions, halide ions, ammonium ions, and a cationic surfactant selected from the group consisting of tetraalkylammonium salts and substituted imidazoline.

This application is directed to the electrodeposition of chromium and more particularly to the use of a surfactant as an ingredient in an improved electrolyte solution.

In recent times substantial improvements have been made in the appearance and the performance of electrodeposited metal coatings, particularly in connection with the deposition of chromium. However, substantial problem and disadvantages still exist in the presently available processes. For example, conventional chromic acid baths deposit the metal at low cathode efficiency and provide coatings having poor covering. Moreover, conventional baths often have poor throwing power. Chromium deposits from conventional baths have been found to be in a highly stressed condition so that they are subject to crack development when the thickness reaches a few hundredths of a milli-inch. Higher current efficiencies, which may approach 40%, can be obtained with aqueous solutions of trivalent compounds but the deposits from such solutions are satisfactory in appearance only when deposited over a very narrow range of pH values. The large amount of hydrogen gas evolved during deposition tends to cause substantial changes in the pH of the solution in the vicinity of the cathode, thus making pH control difficult and restricting the permissible current density range which can be used.

It is recognized by those in the art that considerable economic advantage could be achieved if the current efficiency could be increased. This advantage is particularly attractive with respect to chromium plating baths. It is also recognized that the evolution of hydrogen from the cathode during deposition of the metal is a serious problem and that coatings of improved corrosion resistance and appearance can be provided if the evolution of hydrogen can be controlled. In the past, experimentation with the use of modified chromic acid and trivalent chromium baths has shown little prospect of improvement in the quality of the deposit without a concomitant reduction in current efficiency.

As an improvement over chromium plating from conventional aqueous chromic acid baths, a method has been developed whereby chromium deposits, having greatly improved corrosion resistance and exhibiting a very good appearance, can be provided by electrolytic techniques through the use of a plating bath comprising chromium ions, particularly trivalent chromium ions, and a homogeneous mixture of water and a dipolar organic solvent, preferably aprotic, such as dimethylformamide.

The ratio by volume of water to dimethylformamide

2

may range from 10:90 to 95:5 but preferably between 60:40 and 90:10. These lower concentrations of dimethylformamide make possible a reduction in the cost of the plating bath without necessarily impairing the plating performance.

Solutions containing trivalent metal salts, such as chromic chloride, in combination with organic dipolar solvents and water, may be unstable with respect to composition and plating performance. The physical characteristics of the solution, e.g., color, pH, and viscosity, have been found to change during storage and the color and adhesion of successive metal deposits from the same bath may deteriorate. Moreover, plating baths containing low concentrations of water have a relatively low conductivity, while solutions with higher concentrations of water tend to evolve excessive amounts of hydrogen at the cathode during plating. It has been found that the presence of an ammonium salt improves the stability of the solution and reduces the tendency of the bath to evolve hydrogen at high water content. Moreover the presence of ammonium salts has been found to significantly reduce the effect of changes in pH on the lower limiting plating current density. The ammonium ion should be present at a concentration of at least about 0.2 M and preferably from about 0.6 to about 1 M. At lower concentrations of dimethylformamide, it may be preferable to increase the ammonium ion concentration to above 1 M.

A prerequisite of successful chromium plating from a dipolar organic solvent is that the trivalent chromium ions shall form small moderately stable complexes with the solvent molecule. If there is no complex formation, then the chromic salts are unlikely to be sufficiently soluble. If the complexes formed are excessively stable, then electrodeposition may be difficult. It is believed that the highly electronegative oxygen atoms which characterize the dipolar organic compounds of this invention may act as covalent links in the formation of complexes between the chromic ions and the organic molecules. Such solutions by themselves do not, however, give smooth coherent metallic deposits. The addition of water probably generates the polynuclear olated and oxalated chromic species usually found in solutions of trivalent chromium compounds, which again do not readily give good chromium deposits. The effect of the ammonium ion may be attributed to its structure-disordering properties simplifying the nature of the trivalent chromium in solution, possibly with the formation of mononuclear  $\text{Cr}^{3+}$ -DMF- $\text{H}_2\text{O}$  complexes. The water may be prevented from showing its full protic tendencies by reason of the formation of complexes with the dipolar organic molecules. The halogen ions may be partly solvated, although the ready evolution of chlorine at the anode indicates solvation is not complete.

The pH of the solution should be from 1 to 3.5 and preferably about 2. If the pH is too low, hydrogen tends to be evolved at the cathode in preference to chromium. If the pH is too high, basic chromium compounds are liable to precipitate out. The pH can be adjusted by the use of hydrochloric acid or sodium hydroxide as required.

The current efficiency of the solution may be improved by the addition of boric acid, preferably to a concentration of at least 0.1 M. Boric acid is not normally soluble to the extent of more than about 0.2 M.

In addition to the ammonium ions mentioned above, electroplating baths of the present invention contain a sodium halide which has been found to increase the plating range and current efficiency. Sodium halides are also beneficial in that they enhance the covering power of the bath. It is preferred that the sodium halide be present in a concentration of at least about 0.8 M. Again, however, if lower concentrations of dimethylformamide are

to be used, it may be advantageous to increase the halide ion concentration above 5 M, for example from 7 M to 10 M.

As is pointed out above, it is generally preferable for reasons of economy to utilize solutions having lower DMF concentrations and hence a greater proportion of water. With such solutions, however, certain problems are encountered.

The inclusion of large amounts of chloride and ammonium ions increases the expense, the plating efficiency and current density range may not be very good, and the deposits tend to be dark and in other ways less attractive than those derived from baths with a higher organic content.

In accordance with the present invention, these problems are overcome by adding a surfactant to the plating solution. Although it has been found that a surfactant can improve the plating range at any proportion of water to dipolar organic solvent, it is particularly advantageous at proportions of water to dipolar organic solvent of greater than 60:40 by volume where it enables bright chromium deposits to be obtained under suitable conditions instead of the matt plate produced in the absence of surfactant. Although bright chromium deposits are obtainable from solutions containing as little as 250 g./l. of DMF in the presence of a surfactant, it is preferred that the ratio of water to solvent range between 60:40 and 75:25. The electrolyte will function at lower DMF concentrations but the plating range becomes progressively smaller. At higher DMF concentrations there is no reduction in plating performance but the operating

wherein  $R_1$  is an alkyl having 8 to 18 carbon atoms,  $R_2$ ,  $R_3$  and  $R_4$  are alkyls having from 1 to 2 carbon atoms,  $R_5$  is selected from the group consisting of aliphatic short chain alcohol of the general formula  $C_nH_{2n}OH$  and sodium salt of a carboxylic acid of the general formula



$R_6$  is an alkyl having 9 to 17 carbon atoms,  $R^7$  is an alkylene having 1 to 4 carbon atoms,  $X$  is a halogen selected from the group consisting of bromine, chlorine and iodine and  $n$  and  $n'$  are 1 to 6.

The surfactant should be present in the solution in a concentration of at least 5 p.p.m. and preferably at least 10 p.p.m. Below 5 p.p.m., little or no effect is discernible. The disadvantages of non-ionic and anionic surfactants begin to become discernible at concentrations above 20 p.p.m. There appears to be little or no advantage in using surfactant concentrations above 20 p.p.m., and the use of unnecessary surfactant is undesirable as it causes the bath to foam. However, as will be appreciated, 10 to 20 p.p.m. is a very small amount of surfactant. It is, therefore, preferable to use a cationic surfactant, where the accidental addition of too much to the plating bath does not spoil the chromium deposit.

The invention is illustrated by the following examples. The plating baths employed all contained the following components:

|                   |       |          |     |
|-------------------|-------|----------|-----|
| Chromic chloride  | ----- | M        | 1.4 |
| Ammonium chloride | ----- | Variable |     |
| Sodium chloride   | ----- | M        | 0.8 |
| Boric acid        | ----- | g./l.    | 2   |

TABLE

| Example | NH <sub>4</sub> <sup>+</sup> concentration, M. | Water:DMF, weight ratio | Surfactant                           | Concen- tration, p.p.m. | pH  | Plating range, A./m. <sup>2</sup> | Comments                                                |
|---------|------------------------------------------------|-------------------------|--------------------------------------|-------------------------|-----|-----------------------------------|---------------------------------------------------------|
| 1-----  | 1.0                                            | 60:40                   |                                      |                         | 1.2 | 2,250-160                         | An average result.                                      |
| 2-----  | 1.0                                            | 60:40                   | Na lauryl sulphate                   | 10                      | 1.2 | 2,250-140                         | A slight improvement in range. Black specks in deposit. |
| 3-----  | 1.0                                            | 60:40                   | Cetyl trimethyl ammonium bromide     | 10                      | 1.1 | 2,250-130                         | A good result.                                          |
| 4-----  | 1.0                                            | 60:40                   | do                                   | 15                      | 1.2 | 2,250-120                         | Very good result.                                       |
| 5-----  | 1.0                                            | 60:40                   | do                                   | 30                      | 1.2 | 2,250-130                         | Good but slight frosting at high current density.       |
| 6-----  | 1.0                                            | 60:40                   | Substituted imidazoline <sup>1</sup> | 10                      | 1.2 | 2,250-130                         | Good result.                                            |
| 7-----  | 1.5                                            | 70:30                   |                                      |                         | 1.1 | 2,250-180                         | An average result.                                      |
| 8-----  | 1.5                                            | 70:30                   | Cetyl trimethyl ammonium bromide     | 10                      | 1.1 | 2,250-130                         | As good as the 60:40 bath.                              |
| 9-----  | 1.0                                            | 76:24                   |                                      |                         | 1.1 | 2,250-450                         | Noticeable loss in plating range.                       |
| 10----- | 1.0                                            | 76:24                   | Cetyl trimethyl ammonium bromide     | 10                      | 1.1 | 2,250-475                         | Do.                                                     |

<sup>1</sup> Miranol L2M-SF manufactured by Venture Chemicals Ltd., England, the major constituent of which is



cell voltage, as well as the cost of the electrolyte, increases.

The surfactant may be cationic, anionic, amphoteric or non-ionic, but cationic surfactants are preferred. Non-ionic surfactants tend to give rise to dull deposits, particularly when used in higher concentrations. Anionic surfactants such as Na lauryl sulphate, again particularly at higher concentrations, tend to give rise to black specks on the metal deposits.

Cationic surfactants that may be used according to the invention are tetraalkylammonium salt of the general formula



and substituted imidazoline of the general formula



We claim:

1. An aqueous-dipolar organic solvent electrolyte solution for electrodeposition of chromium on a substrate, said solution comprising a dipolar organic solvent having a high electronegative oxygen atom, water, trivalent chromium ions in a concentration sufficient to permit the electrodeposition of chromium on said substrate, and at least 5 p.p.m. of a surfactant selected from the group consisting of tetraalkylammonium salt of the general formula



and substituted imidazoline of the general formula



wherein  $R_1$  is an alkyl having 8 to 18 carbon atoms,  $R_2$ ,  $R_3$  and  $R_4$  are alkyls having from 1 to 2 carbon atoms,

$R_5$  is selected from the group consisting of aliphatic short chain alcohol having up to 6 carbon atoms of the general formula  $C_nH_{2n}OH$  and sodium salt of a carboxylic acid of the general formula  $C_nH_{2n}OC_{n'}H_{2n'}COONa$ ,  $R_6$  is an alkyl having 9 to 17 carbon atoms,  $R_7$  is an alkylene having 1 to 4 carbon atoms, and X is a halogen selected from the group consisting of bromine, chlorine and iodine, and  $n$  and  $n'$  are 1 to 6, the proportion of water to dipolar aprotic solvent being from about 10:90 to about 90:10.

2. An electrolyte solution according to claim 1 having ammonium ions in a concentration of at least 0.2 M and halogen ions in a concentration at least 0.8 M.

3. An electrolyte solution according to claim 2 wherein the dipolar organic solvent is dimethylformamide.

4. An electrolyte solution according to claim 3 wherein the proportion of water to dipolar aprotic solvent is from about 60:40 to about 75:25.

5. An electrolyte solution according to claim 4 having halogen ions in a concentration of at least 5 M.

6. An electrolyte solution according to claim 4 having ammonium ions in a concentration of at least 1 M.

7. An electrolyte solution according to claim 3 wherein  $R_2$ ,  $R_3$  and  $R_4$  are methyl groups.

8. An electrolyte solution according to claim 7 wherein the surfactant is cetyl trimethyl ammonium bromide.

9. An electrolyte solution according to claim 3 having

between about 5 p.p.m. and about 20 p.p.m. of said surfactant.

10. An electrolyte solution according to claim 3 having said surfactant in a concentration of between 5 p.p.m. and such amount as causes foaming of the electrolyte solution.

11. An electrolyte solution according to claim 3 having ammonium ions in a concentration of between about 0.6 M and about 1 M.

12. An electrolyte solution according to claim 3 wherein the halogen is chlorine.

13. An electrolyte solution according to claim 3 having a pH between about 1 and 3.5.

15

#### References Cited

##### UNITED STATES PATENTS

|           |         |                     |        |
|-----------|---------|---------------------|--------|
| 2,750,335 | 6/1956  | Brown et al. -----  | 204—51 |
| 3,341,434 | 9/1967  | Passal -----        | 204—51 |
| 3,423,297 | 6/1969  | Van der Horst ----- | 204—51 |
| 3,706,641 | 12/1972 | Huba et al. -----   | 204—51 |

##### FOREIGN PATENTS

|           |        |                     |        |
|-----------|--------|---------------------|--------|
| 1,144,913 | 3/1969 | Great Britain ----- | 204—51 |
| 262,033   | 6/1970 | U.S.S.R. -----      | 204—51 |

GERALD L. KAPLAN, Primary Examiner

25